

# United States Patent Office

3,312,552

Patented Apr. 4, 1967

1

3,312,552  
SPOT PREVENTION IN LIGHT-SENSITIVE SILVER  
HALIDE EMULSION LAYERS

Wolfgang Müller-Bardorff, Cologne, and Rolf Behr, Leverkusen, Germany, assignors to Agfa Aktiengesellschaft, Leverkusen, Germany, a corporation of Germany

No Drawing. Filed Aug. 10, 1964, Ser. No. 388,669  
Claims priority, application Germany, Aug 24, 1963,

A 43,888

6 Claims. (Cl. 96—94)

10

This invention relates to improved photographic materials comprising at least one light-sensitive silver halide emulsion layer which material has added thereto special compounds capable of reducing or inhibiting the formation of spots or stains in the processed silver halide emulsion layer, due to the presence of dust particles of metals or metal compounds.

The manufacture and processing of photographic material should be effected with complete exclusion of dust. Consequently, provision is made in the art to free the drying air from dust particles by filtration. Despite precautionary measures, however, it is not possible completely to prevent dust particles being deposited, more especially during the manufacture of the photographic material, and these particles become visible as dark or light spots on the processed photographic material, depending upon whether their action is sensitizing or desensitizing.

Particularly fine particles of metals or metal compounds especially oxides, for example, of iron, aluminium, chromium, nickel or copper, are very disturbing in this respect. Various types of additives have been proposed in the literature to prevent such disturbances. For example, British Patent 623,448 describes aldoximes, which are added to the developer solution or the emulsion in order to take up copper ions. It is further described to utilize acyloins, alkali metal pyrophosphates, metaphosphates, tripolyphosphates and hexametaphosphates, alkali metal oxalates, tartrates, silicates, carbonates and bicarbonates, tungstates, rhenates, osmates, molybdates, chromates and derivatives of ethylene diamine tetracetic acid for restricting the spot or stain formation due to dust particles.

The above compounds are, however, of limited utility since they are either effective only with certain emulsions or since they deleteriously affect photographic or mechanical properties of the photographic material.

It is therefore an object of the present invention to provide antistain agents which have no deleterious effect on photographic materials and which prevent the formation of stains or specks due to the action of dust particles. A further object is to provide photographic silver halide emulsion layer containing those antistain agents. Other objects will appear from the following description of our invention.

The above objects are accomplished by adding to a silver halide emulsion layer of a photographic material a derivative of o-hydroxybenzylamine, the amino group of which is substituted by 2 alkyl radicals containing carboxy groups. The carboxyl substituted alkyl radical having preferably up to 5 carbon atoms.

Particular utility is exhibited by compounds embraced by the following formula:



2

wherein

X and Y each represent hydrogen, halogen such as chlorine or bromine, an alkyl radical, preferably up to 3 carbon atoms such as methyl, ethyl or propyl, a nitro group or a sulphonic acid group, an alkoxy radical having preferably up to 3 carbon atoms, such as methoxy or ethoxy, carboxyl, or the radical



15 Z stands for hydrogen, halogen such as chlorine or bromine, an alkyl radical, preferably up to 3 carbon atoms such as methyl, ethyl or propyl, a nitro group or a sulphonic acid group, an alkoxy radical having preferably up to 3 carbon atoms, such as methoxy, ethoxy or carboxyl;

R<sub>1</sub> and R<sub>2</sub> each represent a carboxyalkyl radical preferably having up to 5 carbon atoms, or salts of the said carboxyalkyl radical.

The compounds according to the invention are added to the photographic emulsions in quantities from 0.1 g. to 15 g. per mol of silver halide. The compounds are preferably added as an aqueous solution of their alkali salts to the photographic emulsions which are ready for casting.

30 Suitable compounds are, for example:





The compounds used according to the invention can be prepared by known processes, for example, as described in *Helv. Chim. Acta*, 1952, 35, 1785-93, and *C.A.*, 1954, 48, 6722.

By way of example, Compound IV is obtained as a sodium salt by reacting o-vanillin with glycine, hydrogenating the Schiff's base which is formed with Raney nickel and reacting the product with sodium chloroacetate.

Compound VI is obtained as a sodium salt by reacting 2-hydroxy-5-nitrobenzylchloride with aminobutyric acid and reacting the product with sodium chloroacetate.

The antistain agents of the present invention are preferably added to the silver halide emulsion. They can, however, also be added to other layers of the photographic elements, such as protective layers, filter layers, antihalation layers and baryta coatings.

The present invention is not restricted to any special silver halide emulsions. The silver halide may consist of silver chloride, silver bromide, silver iodide or mixtures thereof. The emulsions can be optically or chemically sensitized according to any accepted manner. The emulsions may further contain color coupler, stabilizers, coating aids and other additives, which are commonly used in the art.

The following example serve to illustrate the present invention.

#### Example 1

An ordinary photographic silver bromide emulsion which contains 42 g. silver bromide per kg. of emulsion is divided into several portions. Various antistain agents were then added in solution in water in the amounts indicated in the following table. The various portions of the emulsions were then coated at pH 7 on a supported gelatin layer containing dust particles of iron (fine particles of ferrum reductum). The dried coatings were then exposed and developed for about 5 minutes in a photographic developer having the following composition:

|                                                    | G.   |
|----------------------------------------------------|------|
| p-Methylaminophenol                                | 3.5  |
| Hydroquinone                                       | 9.0  |
| Potassium metabisulfite                            | 0.1  |
| Sodium sulfite (anhydrous)                         | 60   |
| Sodium carbonate (anhydrous)                       | 40   |
| Potassium bromide                                  | 4.0  |
| Sodium metaphosphate                               | 4.0  |
| Disodium salt of ethylene diamine tetraacetic acid | 0.25 |
| Water to make one liter.                           |      |

The dust particles cause the formation of black spots surrounded by halos on the processed photographic element. The results are given in the following table:

TABLE 1

| Sample | Addenda per kg. of emulsion                                                               | Relative number of black stains |
|--------|-------------------------------------------------------------------------------------------|---------------------------------|
| 5 A    | Standard                                                                                  | 100                             |
| B      | 3 ml. of a 25% aqueous solution of the disodium salt of Compound VII.                     | 0                               |
| C      | 5 ml. of a 25% aqueous solution of the disodium salt of ethylenediamine tetraacetic acid. | 20                              |
| 10 D   | 10 ml. of a 10% aqueous solution of the sodium salt of 2-hydroxy-5-sulfo benzoic acid.    | 70                              |
| E      | 200 ml. of a 2% aqueous solution of the sodium salt of 2-hydroxy-benzylamino acetic acid. | 20                              |

#### Example 2

An ordinary photographic silver bromide emulsion which contains 42 g. silver bromide per kg. of emulsion is divided into several portions. Various antistain agents were then added in solution in water in the amounts indicated in the following table. The various portions of the emulsions were then coated at pH 7 on a supported gelatin layer containing dust particles of iron (fine particles of ferrum reductum). The dried coatings were then exposed and developed for about 5 minutes in the photographic developer described in Example 1.

The dust particles cause the formation of black spots surrounded by halos on the processed photographic element. The results are given in the following table:

TABLE 2

| Sample | Addenda per kg. of emulsion                                              | Relative number of black stains |
|--------|--------------------------------------------------------------------------|---------------------------------|
| 35 A   | Standard                                                                 | 100                             |
| B      | 0.7 g. of the sodium salt of Compound I (dissolved in 5 ml. of water).   | 0                               |
| C      | 0.7 g. of the sodium salt of Compound VII (dissolved in 3 ml. of water). | 0                               |

#### Example 3

An ordinary photographic silver bromide emulsion which contains 63 g. of silver bromide per kg. of emulsion is divided into several portions. Various antistain agents were then added in solution in water in the amounts indicated in the following table. The various portions of the emulsions were then coated at pH 5.8-5.9 on a supported gelatin layer containing dust particles of iron (fine particles of ferrum reductum). The dried coatings were then exposed in the photographic developer composition described in Example 1.

The dust particles cause the formation of black spots surrounded by halos on the processed photographic element. The results are given in the following table:

TABLE 3

| Sample | Addenda per kg. of emulsion                                         | Relative number of black stains |
|--------|---------------------------------------------------------------------|---------------------------------|
| 60 A   | Standard                                                            | 100                             |
| B      | 7 ml. of a 10% aqueous solution of the sodium salt of Compound VII. | 0                               |

#### Example 4

An ordinary photographic silver bromide emulsion which contains 83 g. silver bromide per kg. of emulsion is divided into several portions. Various antistain agents were then added in solution in water in the amounts indicated in the following table. The various portions of the emulsions were then coated at pH 6.5 on a supported

gelatin layer containing dust particles of iron (fine particles of ferrum reductum). The dried coatings were then exposed in the photographic developer composition described in Example 1.

The dust particles cause the formation of black spots surrounded by halos on the processed photographic element. The results are given in the following table:

TABLE 4

| Sample | Addenda per kg. of emulsion                                                                | Relative number of black stains |
|--------|--------------------------------------------------------------------------------------------|---------------------------------|
| A..... | Standard.....                                                                              | 100                             |
| B..... | 0.5 g. of sodium salt of ethylenediamine tetra-acetic acid (dissolved in 20 ml. of water). | 30                              |
| C..... | 0.5 g. of Compound VII.....                                                                | 0                               |

## Example 5

2 silver bromide emulsions, the one containing 80 g. of silver bromide per kg. of emulsion and the other 130 g. of silver bromide per kg. of emulsion are divided in several portions. Various antistain agents are added in solution in water in the amounts indicated in the following table. The various portions of the emulsions are then coated at a pH of 6.7 each on 1 side of a transparent transport of cellulose acetate which is coated on each side with a gelatin layer containing fine particles of rust and iron. The resulting photographic material is processed as described in Example 1.

The results of the comparison tests are given in the following table:

TABLE 5

| Sample | Addenda per kg. of emulsion                                     | Relative number of black stains |
|--------|-----------------------------------------------------------------|---------------------------------|
| A..... | Standard.....                                                   | 100                             |
| B..... | 0.5 g. of the sodium salt of ethylenediamine tetra-acetic acid. | 40                              |
| C..... | 0.5 g. of Compound VII.....                                     | 0                               |

We claim:

1. A photographic material containing at least one supported light-sensitive silver halide emulsion layer, the said material contains as an antistain agent an effective amount of an o-hydroxybenzylamine, the amino group of which is substituted by 2 alkyl radicals containing carboxyl groups.

2. A photographic material as defined in claim 1, containing as an antistain agent an effective amount of a compound having the following formula:



45

50

55

wherein

$\text{R}_1$  and  $\text{R}_2$  each represent a carboxyalkyl radical having up to 5 carbon atoms;  
 $\text{X}$  and  $\text{Y}$  each represent a member of the group consisting of hydrogen, halogen, alkyl, nitro, sulfo, alkoxy, carboxyl and a radical of the following formula



$\text{Z}$  stands for a substituent of the group consisting of hydrogen, halogen, alkyl, nitro, sulfo, alkoxy, ethoxy and carboxyl.

3. A photographic material as defined in claim 2, containing as an antistain agent an effective amount of the following compound:



25

4. A photographic material as defined in claim 2, containing as an antistain agent an effective amount of the following compound:



30

5. A photographic material as defined in claim 2, containing as an antistain agent an effective amount of the following compound:



45

6. A photographic material as defined in claim 2, containing as an antistain agent an effective amount of the following compound:



50

No references cited.

NORMAN G. TORCHIN, Primary Examiner.

60 C. E. DAVIS, Assistant Examiner.